

## UNITED STATES PATENT OFFICE.

EDWIN CORNING, OF KENWOOD, AND PERCY A. E. ARMSTRONG, OF LOUDONVILLE,  
NEW YORK.

## ALLOY STEEL FOR METAL-CUTTING TOOLS.

No Drawing. Continuation of application Serial No. 420,432, filed October 29, 1920. This application filed January 5, 1922. Serial No. 527,223.

*To all whom it may concern:*

Be it known that we, EDWIN CORNING, a citizen of the United States, and a resident of Kenwood, county of Albany, and 5 State of New York, and PERCY A. E. ARMSTRONG, a subject of the King of Great Britain, and a resident of Loudonville, county of Albany, and State of New York, have invented a new and useful Improvement 10 in Alloy Steel for Metal-Cutting Tools, of which the following is a specification.

This invention relates to alloy steel for metal cutting tools, having properties generally intermediate between carbon steel 15 and high-speed steel.

The present application is a continuation of our co-pending application Serial No. 420,432, alloy steel for metal cutting tools, filed Oct. 29, 1920.

For small metal cutting tools, such as drills, taps, reamers and the like, carbon steel answers sufficiently well, takes a keen cutting edge and produces smooth finished 25 work, but is limited in its application, because under heat it softens and dulls rapidly.

High speed steel, which is commonly used for somewhat larger drills and similar tools 30 which have to withstand greater heat, is not, of course, rapidly softened by frictional heat, but, in addition to its high price, has the objection that the work produced is not so smooth and well finished as can be obtained by sharp edge carbon steel tools, for 35 example, and a subsequent separate finishing operation is usually required. For example, drilled holes require finish reaming to produce satisfactory work. Furthermore, in the case of taps, for example, the 40 teeth of the tap are often injured by the high temperatures required for heat treatment of high speed steel.

The present invention relates to the provision 45 of an alloy steel having the desirable properties of both carbon steel and high speed steel, that is, which will retain a hard, keen cutting edge and which is very strong, and at the same time will 50 not soften when drawn to medium tem-

peratures, such as 500-700° F. The steel of the present invention contains chromium, vanadium and molybdenum, and also contains silicon considerably in excess of the usual silicon content of steel, silicon being 55 present in our improved alloy steel preferably to the extent of from about .5% to 2.5%. When made into tools for cutting metal, such as drills, taps, reamers and the like, it can be used for the production of 60 smooth, finished work without the necessity for separate finishing operations, and does not require heat treatment at such high temperatures as in the case of high speed steel, so that there is practically no tendency for 65 any burning off of the tips of the teeth of taps and similar tools during heat treatment. This steel has other features of advantage as will appear from the following description.

An important feature of the invention relates to the employment of silicon as one of the components of the alloy. The silicon appears to serve as a sort of solvent for other components, and causes them to form 75 a chemical combination with one another and produces an alloy steel having improved properties. A second function of the silicon is to raise the transformation point of the resulting alloy, thus imparting 80 to the alloy steel the very valuable property of hardening at relatively high temperatures. A third function of the silicon is to enhance the air hardening properties 85 of the alloy. Silicon enables the chromium and molybdenum in combination with the carbon and iron to take on a tremendously enhanced air hardening property. It also prevents the breaking down of this hard state when being drawn at temperatures 90 which would cause a straight chromium, carbon or chromium-molybdenum-carbon steel to soften.

According to another feature, an alloy steel is provided having as one of its components a predetermined proportion of vanadium. This alloy steel has an increased red hard property. The use of vanadium also creates a lag to transformation, that is to say, when the steel is reheated for a 100

very short period after being quenched for hardening, it is given the quality of having a lag to the breaking down of the solid solution produced in quenching. Consequently, cutting tools made of the alloy so made can withstand overheating of their cutting edges for limited times without destruction of their cutting ability.

According to another feature, an alloy steel is provided having as one of its components a predetermined proportion of cobalt. This alloy steel has qualities of the same general character as the vanadium alloy steel just described, to a different degree.

According to still another feature, an alloy steel is provided having neither vanadium or cobalt, but in which there is employed carbon, molybdenum, chromium, silicon and other components. The carbon gives desirable mineral hardness to the alloy, which may be enhanced by other components. The molybdenum in combination with the carbon and iron adds to the hardness and improves other desirable physical qualities. Chromium in combination with the molybdenum and carbon adds materially to the air hardening effect of such combination.

One example of a composition for an alloy steel in accordance with the present invention is as follows:

|                      | Per cent. |
|----------------------|-----------|
| Carbon               | .50       |
| Chromium             | 1.50      |
| Molybdenum           | 1         |
| Manganese            | .40       |
| Silicon              | 1.50      |
| Vanadium             | .75       |
| Cobalt approximately | 1         |

Balance iron with small amounts of phosphorus and sulfur.

In order to harden this alloy it is heated as quickly as possible to substantially 1900° F., without quenching in oil or water. Variations in manganese in this alloy will require inverse variations in the temperature to which the alloy is heated; for example, if the manganese is increased to 1% the temperature should be changed to substantially 1500° F., while if the manganese is increased to 1.5% the temperature should be reduced to substantially 1450° F.

Another example of an alloy made in accordance with the present invention is of about the following composition:

|            | Per cent. |
|------------|-----------|
| Carbon     | 1         |
| Chromium   | 2         |
| Molybdenum | 2         |
| Manganese  | .40       |
| Silicon    | 1         |
| Vanadium   | 1         |
| Cobalt     | 1         |

Balance iron with small amounts of phosphorus and sulfur.

In order to harden this alloy it should be heated as quickly as possible to substantially 1800° F., and quenched in oil or water. Variations in manganese require variations in the heat treatment temperature as in the preceding example.

A third example of an alloy made in accordance with the present invention is of about the following composition:

|            | Per cent. | 75 |
|------------|-----------|----|
| Carbon     | 1.50      |    |
| Chromium   | 2         |    |
| Molybdenum | 2         |    |
| Manganese  | .40       |    |
| Silicon    | 2         | 80 |
| Vanadium   | .50       |    |
| Cobalt     | 2         |    |

Balance iron with small amounts of phosphorus and sulfur.

The heat treatment of this alloy consists of heating to substantially 1800° F., as quickly as possible and quenching in oil or water. Selection of the heat treatment temperature is made in accordance with variations in percentage of manganese as in the preceding examples.

Another example of alloy made in accordance with the present invention is of about the following composition:

|            | Per cent. | 95  |
|------------|-----------|-----|
| Carbon     | .50       |     |
| Chromium   | 10        |     |
| Molybdenum | 5.75      |     |
| Manganese  | .40       |     |
| Silicon    | 2.5       | 100 |
| Vanadium   | 2         |     |
| Cobalt     | 2         |     |

Balance iron with small amounts of phosphorus and sulfur.

In the heat treatment of this alloy heat should be applied until the alloy has a temperature of substantially 2100° F. The alloy should then be cooled in the air. This alloy may be cast for use in forming cutting tools.

More or less variation is possible without any substantial detriment to the desirable qualities of the material and good results are obtained with varying quantities of the several components within substantially the following range:

|            | Per cent. |
|------------|-----------|
| Carbon     | .25-2     |
| Molybdenum | .50-5.75  |
| Silicon    | .50-2.5   |
| Chromium   | .50-10    |
| Vanadium   | 0-2       |
| Manganese  | 0-1.5     |
| Cobalt     | 0-2       |

Balance iron with small amounts of phosphorus and sulfur.

This represents about the outside limits, but good results may be obtained with smaller proportions of some of the alloy com-

ponents, with composition about as follows: carbon .25-2%, molybdenum .50-2%, silicon .50-2%, chromium .50-2%, vanadium up to 1%, manganese up to 1%, cobalt up to 1%, and the balance principally iron.

We have found that good results are obtained with heat treatment of alloys made in accordance with the present invention, which consists of heating the alloy to a temperature of approximately 1800° F., in as short a time as possible, after which the alloy may be air hardened or quenched in oil or water. It is preferably not held at this temperature more than a half-minute or so longer than necessary to heat the piece throughout.

Another alloy steel may comprise, for example, components within substantially the following range:

|            | Per cent. |
|------------|-----------|
| Carbon     | .25-2     |
| Molybdenum | .50-.75   |
| Silicon    | .50-2.5   |
| Chromium   | .50-10    |
| Vanadium   | .25-2     |
| Manganese  | 0-1.5     |

Balance iron with small amounts of phosphorus and sulfur.

Heat treatment substantially as given for previously described alloy steels.

The cobalt steel may comprise, for example, components within substantially the following range:

|            | Per cent. |
|------------|-----------|
| Carbon     | .25-2     |
| Molybdenum | .50-.75   |
| Silicon    | .50-2.5   |
| Chromium   | .50-10    |
| Manganese  | 0-1.5     |
| Cobalt     | .25-2     |

Balance iron with small amounts of phosphorus and sulfur.

Another modification comprises components within substantially the following range:

|            | Per cent. |
|------------|-----------|
| Carbon     | .25-2     |
| Molybdenum | .50-.75   |
| Silicon    | .50-2.5   |
| Chromium   | .50-10    |
| Manganese  | 0-1.5     |

Balance iron with small amounts of phosphorus and sulfur.

The steel works well in the mill, is substantially free from seams, and can be cast into very smooth ingots. In rolling the temperature should not be carried unduly high and should preferably be kept under

2100° F. After rolling the steel should preferably be cooled slowly as, for example, in lime, thereby removing strains which may result from rapid cooling. This becomes more important as the alloying constituents are increased. The steel will anneal and

becomes quite easy to machine when properly annealed. There is very little tendency for this alloy combination to move, that is to say, to exhibit tendency to warping, or other malformation upon heating up and quenching, which is a feature of great advantage in heat treatment of tools. The characteristic grinding spark given off in grinding articles made of our improved alloy steel, which does not contain tungsten, is markedly different from the tungsten colored spark. This is a feature of marked advantage both in manufacture and use, as this alloy steel can be readily distinguished from high speed steels by observation of the spark produced upon grinding. The foregoing applies whether the alloy steel is in the annealed or hardened state.

We claim:

1. As a new composition of matter, an alloy steel of analysis having substantially the following range: carbon .25-2%, chromium .50-10%, molybdenum .50-.75%, silicon .50-2.5%, vanadium 0-2%, manganese 0-1.5%, cobalt 0-2%, and the principal part of the remainder iron.

2. Metal cutting tools made from alloy steel as claimed in claim 1.

3. Drills for drilling metal made from alloy steel as claimed in claim 1.

4. As a new composition of matter, an alloy steel of analysis having substantially the following range: carbon .25-2%, molybdenum .50-.75%, silicon .50-2.5%, chromium .50-10%, vanadium .25-2%, manganese 0-1.5%, and the principal part of the remainder iron.

5. Metal cutting tools made from alloy steel as claimed in claim 4.

6. Drills for drilling metal made from alloy steel as claimed in claim 4.

7. As a new composition of matter, an alloy steel of analysis having substantially the following range: carbon .25-2%, molybdenum .50-.75%, silicon .50-2.5%, chromium .50-10%, manganese 0-1.5%, cobalt .25-2%, and the principal part of the remainder iron.

8. Metal cutting tools made from alloy steel as claimed in claim 7.

9. Drills for drilling metal made from alloy steel as claimed in claim 7.

10. As a new composition of matter, an alloy steel of analysis having substantially the following range: carbon .25-2%, molybdenum .50-.75%, silicon .50-2.5%, chromium .50-10%, manganese 0-1.5%, and the principal part of the remainder iron.

11. Metal cutting tools made from alloy steel as claimed in claim 10.

12. Drills for drilling metal made from alloy steel as claimed in claim 10.

13. An air hardening alloy steel adapted to withstand temperatures of about 500-700° F., without material softening, of analysis

within substantially the following range: 15. Drills for drilling metal made from carbon .25-2%, chromium .50-2%, molybde- alloy steel as claimed in claim 13. num .50-2%, silicon .50-2%, vanadium up In witness whereof, we have signed our 10 to 1%, manganese up to 1%, cobalt up to names hereto.

5 1%, and the balance principally iron.

14. Metal cutting tools made from alloy steel as claimed in claim 13.

PERCY A. E. ARMSTRONG.  
EDWIN CORNING.